

Feb. 20, 1934.

H. D. MATTHEWS

1,948,121

BIMETALLIC ELEMENT

Filed March 23, 1932

SILICON-COPPER ALLOY

NICKEL-STEEL ALLOY OR EQUIVALENT

INVENTOR.  
HOWARD D. MATTHEWS

BY

*Howard D. Matthews*

ATTORNEY.

## UNITED STATES PATENT OFFICE

1,948,121

## BIMETALLIC ELEMENT

Howard D. Matthews, Detroit, Mich., assignor  
to W. M. Chace Valve Company, Detroit,  
Mich., a corporation of Michigan

Application March 23, 1932. Serial No. 600,642

9 Claims. (Cl. 297—15)

This invention relates to bimetallic elements, and the object is to secure a bimetallic element particularly adaptable for low temperature applications in which the element is not heated to temperatures materially in excess of four hundred degrees Fahrenheit.

A bimetallic element for low temperature applications has heretofore been made of brass and invar secured together but brass is not suitable for hot rolling after being welded to the invar or nickel-steel side of the blade to secure the desired thinness of blade and further the brass and invar bimetal frequently takes a permanent set in service. Also, when bimetal is formed into various shapes as may be required for its specific application, a heat treatment is required to relieve the stresses set up by rolling as well as that produced in the forming operation. Invar and other nickel steel alloys require a temperature of about 700 degrees F. to age the steel at which temperature the brass element would be softened. Therefore the present practice in the manufacture of the brass-invar bimetal is to heat treat the element at about 350 degrees F., under which temperature the brass is properly aged but the nickel steel side has not been relieved of the internal stresses. As a result of such latter treatment of the brass-invar element, stresses in the nickel steel or invar side cause a change in position of the element thereby introducing inaccuracies in action of the blade under variation in temperatures.

I have devised a bimetallic blade in which both elements thereof require or may be subjected to heat treatment at approximately the same temperature to properly age the same and therefore by my invention I have secured a bimetal that can be properly heat treated to give greater accuracy in service and also as a resultant feature of my invention I have secured an element operable in all situations in which the brass-invar has heretofore been used and in which the stresses may be relieved by heat treatment set up by hot rolling as well as in the final forming for any specific use and a bimetal in which the element having the higher coefficient of expansion (usually termed the "high side") is suitable for hot rolling after being welded to the nickel steel or invar element (usually termed the "low side") thereby reducing factory costs below that involved in the production of the commonly known brass-invar bimetal.

These and various other objects and features

of the invention and the manner in which they may be attained as is hereinafter more fully described and claimed.

The accompanying drawing is a representation of a bimetallic element showing a strip of nickel-steel alloy fused throughout its length to a similar strip of silicon copper alloy.

In the production of my new bimetallic element I preferably use a nickel steel alloy as has heretofore been commonly used in this art for the low side of a bimetallic blade, and it is to be noted that the nickel content of this nickel-steel element may be varied from approximately 36 per cent to approximately 42 per cent to secure the desired action of the blade for any specific application.

The invention, however, is not confined to the use of a nickel-steel alloy as the element having the lower coefficient of expansion as any metal or composition of metal adaptable for use as the "low side" may be used providing it may be aged by heat treatment at the same temperature as the "high side" herein described. For the high expansion side, which has heretofore been the element causing difficulty in manufacture of the brass-invar couple as above outlined, I use a composition consisting of the following ingredients in approximately the following percentages, viz:

|         |                  |
|---------|------------------|
| Silicon | 2 per cent       |
| Tin     | 1½ to 2 per cent |
| Copper  | 96 per cent      |

This alloy is essentially pure copper with small amounts of alloying elements as silicon and tin. Cadmium may be used in the percentage of about .005 in the above composition to increase the ability of the alloy to be properly processed and incidentally to make it less corrosive and the cadmium can also be used in place of one or the other of said alloying elements. This composition has a coefficient of expansion of .000010 per degree F. corresponding very closely to the coefficient of expansion of commercial bronze.

The silicon content of the high expansion member of the bimetallic element is used to harden the copper and while 2 per cent silicon to 96 per cent copper has been found preferable, the silicon content may be as high as about 5 per cent. The purpose of the silicon is to harden the copper and it has been found in my experience that the subjection of the silicon-copper member of the element to heat tends to increase the hardness of the copper.

as the temperature is increased and thus better adapts the same for use in conjunction with a low expansion element formed of a nickel-steel alloy having a nickel content within the range 5 of 36 per cent to 42 per cent. In each of these two members of the thermostatic couple it is necessary to subject the same to a temperature of about 700 degrees F. to affect molecular change and to relieve the same of the internal 10 strains which might affect operation of the element in use at lower temperatures and it is this feature which forms one of the principal objects of my invention, namely, to secure a bimetallic blade or element each member of 15 which has such physical characteristics that molecular change takes place and each member is thereby relieved of internal stress, inherent therein or caused in the formation of the blade, by heat treating at the same temperature. The tin and/or cadmium content reduces the tendency to corrode and also makes the composition more ductile and therefore more readily cut or tooled in manufacture of 20 the blade.

25 It has heretofore been known that a desirable thermostatic element consisting of two metal alloys of dissimilar thermal characteristics may be formed by placing the same in a clamp or press of the proper shape and held under mechanical strain and heating the same to temperature above that to which it may be subjected in use to relieve the element of such internal stresses as might affect its operations 30 at lower temperatures. Such previous known method of formation of a bimetallic element however is expensive due to the labor cost involved in placing the same in forms under mechanical stress and therefore by my invention I have reduced the cost of manufacture to a 35 material degree and have further achieved a more satisfactory acting bimetallic element for use under certain degrees of temperature as molecular change has been produced in both members of the element in subjecting the same 40 to a higher degree of heat subsequent to formation thereof than it will be subjected to in use and have also lessened the cost of manufacture in that I have found that for some uses the heat treatment need not necessarily be as 45 high as will be required for such elements as are to be subjected to certain higher temperatures in use. Therefore by my invention and through choice of any two metals or alloys of 50 metals adaptable to serve as the opposing members in a bimetallic element and having such physical characteristic that internal stress is relieved in both elements by heat treatment at the same temperature, I can produce a bimetallic blade that in its field of service is unaffected in its accuracy of operation due to the 55 presence of internal strains in either member of the couple.

60 The bimetal is formed of sheets of silicon-copper alloy and nickel-steel welded or otherwise secured together to form a couple inseparable by heat to which the blade is subjected in use and provides a blade that is as sensitive to temperature change as is the usual brass-invar bimetal element commonly known to the trade and may replace such elements in the usual installations in which it is found.

65 My improved bimetal may be heat treated as previously stated to relieve the internal stresses resulting from the hot rolling to the desired 70 thickness in manufacture subsequent to the

welding of the sheets together and to also relieve stresses set up by any forming operations to which the element may be subjected. I therefore, by use of the herein specified composition for the "high side" in conjunction with 75 any of the metals now used in conjunction with brass for the "low side", have secured a more highly efficient bimetal for use within a temperature range up to approximately 400 degrees F. that avoids troubles arising in the use of 80 brass and nickel steel or invar couple due to the metal having been relieved of the internal stresses caused by rolling or forming operation and therefore avoid the inaccuracies in operation of previously known bimetallic elements 85 commonly provided for use within the temperature range stated.

It is also to be noted that, while I have above dwelt upon the characteristics of my improved bimetal for hot rolling, this metal may be cold 90 rolled without any danger of cracking. Brass becomes brittle with cold rolling and also cannot be hot rolled and my new bimetal therefore is superior to the previously well known brass-invar bimetal in that it may be either cold rolled 95 or hot rolled as may be desired.

It is also to be noted that a blade formed of silicon-copper and nickel-steel couple has a much greater activity than the brass invar or Monel metal nickel-steel couple of the prior art 100 and is less costly than the Monel metal "high sides" often used. This higher degree of activity is of great importance in a bimetallic element for use in what is termed the low temperature field and, in addition to its characteristic of responding to heat treatment in relief of internal stress to approximately the same degree as the nickel-steel alloy with which it is associated, has the further characteristic of not thinning out 105 so rapidly in the rolling process as the brass or bronze elements heretofore used in bimetal blades for low temperature work.

Having thus briefly described my invention, what I claim and desire to secure by Letters Patent of the United States is—

1. A bimetallic element comprising two elements of dissimilar thermal characteristics, one of said elements being a silicon-copper alloy containing 2 per cent silicon and 96 per cent copper and having a comparatively high coefficient of expansion and the other a nickel-steel alloy having a comparatively low coefficient of expansion, the silicon-copper alloy being directly welded to the nickel-steel alloy and having the characteristic of responding to heat 110 treatment for relief of internal stresses developed in the formation of the element approximately the same as the nickel-steel alloy.

2. A bimetallic blade comprising two metal members of dissimilar thermal characteristics 115 welded together and hot rolled to the desired thickness, the element of higher thermal characteristic containing about 2 per cent silicon and 96 per cent copper and the element of lower thermal characteristic being a nickel-steel alloy 120 having a nickel content within the range of from 36 per cent to 42 per cent, both said elements responding practically alike to heat treatment for relieving internal stresses developed in manufacture of the blade, the element of higher 125 thermal characteristic having a coefficient of expansion of approximately .000010 per degree Fahrenheit and the other having a lower coefficient of expansion.

3. A heat responsive device comprising two 130

metallic elements, one of the elements being an alloy of approximately 2 per cent silicon, approximately 96 per cent copper and approximately 2 per cent tin and having a comparatively high coefficient of expansion and the element having the lower coefficient of expansion being a nickel-steel alloy of approximately 36 to 42 per cent nickel content.

4. A heat responsive device comprising two metallic elements fused together, one of the elements being an alloy of approximately the following composition, viz:

Silicon..... 2 per cent  
15 Tin..... 1½ per cent  
Copper..... 96 per cent  
Cadmium..... Approximately ½ of 1 per cent

and the other element being a nickel-steel alloy having a nickel content within the range of 20 from 36 per cent to 42 per cent.

5. A heat responsive device comprising two metallic elements fused together, one of the elements being an alloy of approximately the following composition, viz:

25 Silicon..... 2 per cent  
Tin..... Approximately 1½ per cent  
Copper..... 96 per cent  
Cadmium..... Approximately ½ of 1 per cent

30 and the other element being a nickel-steel alloy containing approximately 36 per cent nickel.

6. A heat responsive device comprising two metallic elements fused together and of a relative thickness greater than the thickness desired in the final element, then submitting the same to a rolling operation to reduce the same to the desired final thickness, one of the elements being an alloy of approximately the following composition:

40 Silicon..... 2 per cent  
Tin..... 2 per cent  
Copper..... 96 per cent

45 and having a coefficient of expansion of approximately .000010, the other element being a nickel-steel alloy containing approximately 36 per cent nickel and having a lower coefficient of expansion.

50

7. A heat responsive device comprising two metallic elements of different coefficients of expansion fused together, the element having the higher coefficient of expansion consisting of approximately 96 per cent copper and 4 per cent of alloying elements such as ½ of 1 per cent tin, 2 per cent silicon and cadmium to secure ductility and non-corrosiveness of the element, and the element having the lower coefficient of expansion being a nickel-steel alloy having a nickel content within the range of approximately 36 to 42 per cent.

8. A bimetallic element comprising two metal members of dissimilar thermal characteristics welded together and adapted to act as a unit in response to temperature change, the member of higher coefficient of expansion being a silicon-copper alloy substantially as specified and the element of lower coefficient of expansion being a nickel-steel alloy substantially as specified, each of the said members having such physical characteristics that internal molecular stress existent therein is relieved on subjection to a temperature of approximately 700 degrees F. whereby the unit, subsequent to its formation, may

85 be heat treated to free the same from internal strains affecting operation thereof as a unit at temperatures below 700 degrees F.

9. A bimetallic element comprising two metal members of dissimilar thermal characteristics secured together and adapted to act as a unit in response to variations in temperature within the range below that productive of molecular change, both said members having such physical characteristic that molecular change takes

105 place therein and each is relieved of internal stress while in a mechanically unrestrained state through subjection to a temperature higher than that to which it is to be subjected in use, said element subsequent to being formed being 110 subjected to the high temperature whereby the heat treated element is freed of internal strains tending to detrimentally affect operation thereof at lower temperatures.

120

90

95

100

105

110

115

120

125

130

135

140

145

150

HOWARD D. MATTHEWS.

55

60

65

70

75